

Sept. 27, 1938.

L. PRINZ ET AL

2,131,298

PROCESS FOR THE PHOTOMECHANICAL PRODUCTION OF SINGLE- OR  
MULTICOLOR PICTURES OR WRITING ON HARD MATERIAL  
Filed Feb. 8, 1937

Fig. 1.



Fig. 2.



Fig. 3.



INVENTORS:  
Leopold Prinz  
& Paul Morgenstern,

By Stebbins, Blenko  
& Paulette, Ottys.

## UNITED STATES PATENT OFFICE

2,131,298

## PROCESS FOR THE PHOTOMECHANICAL PRODUCTION OF SINGLE- OR MULTI-COLOR PICTURES OR WRITING ON HARD MATERIAL

Leopold Prinz, London, England, and Paul Morgenstern, Vienna, Austria, assignors to The Primographic Company Limited, London, England, a British company

Application February 8, 1937, Serial No. 124,738  
In Austria February 13, 1936

## 1 Claim. (Cl. 95—5.5)

This invention relates to processes for the photomechanical production of single- or multi-color pictures or writing on hard material.

Numerous proposals have heretofore been made for photomechanically producing single- or multi-color pictures or writing on plates or other articles of hard material, such as glass, Celluloid, or metal. In these processes there is first applied to the plate which is to be provided with pictures or writing a light-hardenable coating which exhibits a differential hardening on exposure to light consisting, for example, of a chromate-albumen layer, after which this layer is exposed to light through a transparency comprising the original to be copied, followed by the application of the respective color. The material thus treated is then developed in water, when the color adheres only to the exposed places, and can be wiped off the other places with the aid of a cotton-wool or similar soft pad.

Known processes of this kind have a number of drawbacks. Particularly, they are extremely tedious since the colors dry only very slowly on the light-hardenable layer. This circumstance makes itself felt more particularly in the production of multi-color pictures or writing, in which, in the manner described, after the exposure of the light-hardenable layer, first one color has been applied, and then, after this color has dried on this layer a further color has then been applied, and so on. For these reasons it has been impossible heretofore to use such processes for rapid and continuous mass production.

A further disadvantage of the known processes is that the outlines of the pictures or writing, or parts thereof, are liable to be not sufficiently sharply defined, or that the pictures give a blurred impression, this being attributable to the fact that it has not been possible hitherto to apply the color absolutely homogeneously. In fact, hitherto the color has been applied either by means of rollers or by spraying. The application of the color by means of a roller is, however, tedious and troublesome; the pressure exerted manually by means of the roller is not uniform at all points and, therefore, ill-defined outlines are formed. The spraying method as practised heretofore, likewise has the disadvantage that the outlines are ill-defined, and, in addition, the colors hitherto found to be suitable for the spraying method, for example aniline dyes, are not always fast to light. The majority of colors capable of being sprayed attack the chromate-albumen layer, or destroy it in parts, so that it has

not proved possible hitherto to obtain satisfactory results even by means of the spraying method. Further, the known processes are attended by the drawback that in the course of development in water or the subsequent treatment with the cotton-wool pad the colors may readily be smudged.

The present invention has for its object to provide an improved process for the photomechanical production of single- or multi-color pictures or writing on hard material, which obviates the described drawbacks.

The invention consists primarily in the employment, for the production of the pictures or writing, of a coloring matter consisting of a fluid dispersion of one or more powdered mineral pigments in a mixture of printer's varnish and petrol or other readily volatile liquid. Powdered mineral pigments are fast to light, and can be sprayed on to the light-hardenable layer in the form of the above dispersion. It will be appreciated that the expression "light-hardenable layer" is used herein to mean only those layers which exhibit a differential hardening on exposure to light.

The powdered mineral pigments are preferably mixed with about 10% of printer's varnish, 30% of petrol and 2% of oil of lavender. Thus, according to the invention, the coloring matter solutions hitherto employed in photomechanical duplicating processes of the described nature are abandoned, and in their place there is employed pulverulent mineral coloring matter (powdered mineral pigment) which is rendered capable of being sprayed by the specified additions. The employment of petrol or of an analogous readily volatile substance has the advantage that this medium evaporates rapidly after the application of the color, so that the color dries very quickly. The addition of printer's varnish causes the powdered mineral pigment to adhere well to the light-hardenable layer. The purpose of the addition of oil of lavender is to obtain a homogeneous, readily sprayable mass of the required consistency.

In some cases, one or more pigments, e. g. in the form of ink, may be added to the mass for varying or modifying the tone or color of the mineral coloring matter.

Any of the layers employed in the previous processes may be used as the light-hardenable layer, preferably a chromate-albumen layer. It has now been found that it is possible, when using powdered mineral pigments, to provide a light-hardenable layer of such composition that the

time required for drying is very considerably reduced. This is achieved by the addition of a 15% alum solution to the chromate-albumen solution before application to the material. The powdered mineral pigment is thereby rapidly absorbed, with the result that the time required for drying is very much reduced. Further, it has been found that the addition of alum to the light-hardenable layer has the effect of making the colors "harder", the latter are not impaired in any way in the course of the development in water and also do not tend to become smudged in the course of the usual treatment with the cotton wool pad. The term "development" refers to the step of rendering the image visible by removal of unhardened parts of the exposed light-sensitive layer by washing with water. Rapidity of drying is thus achieved in the case of the invention by two means, namely by an addition of alum to the light-hardenable coating, and by an addition of petrol to the powdered mineral pigments.

The invention further provides the possibility of obtaining multi-color reproductions in a far simpler manner than hitherto, namely, for example, by spraying on several colors simultaneously, if they are spaced apart, or in succession with the employment of stencils or masks. The application by spraying of a plurality of colors by means of stencils is known in the production of signs when the colors are applied directly, i. e. without the employment of a light-hardenable layer. In the photomechanical processes to which the present invention relates, spraying by means of stencils has not been carried out heretofore, for the reason that in consequence of the colors hitherto employed for this purpose, sharp outlines could not be obtained by means of a spraying process with the aid of stencils. It is only through the employment of powdered mineral pigments in the above-mentioned admixtures that it becomes possible to spray a plurality of colors with the aid of stencils.

It is advisable, in the production of multi-color pictures, to dust the surface with talcum powder after the application of the different colors. The individual colors are thereby prevented from becoming smudged or blurred, or the outlines from running into one another during development.

Copies obtained by the new process may be employed as advertisement signs, makers' name-plates and output-plates, scales more particularly for wireless sets for which high demands are made as regards sharpness of outline, watch and clock glasses, advertising mirrors, and other advertisement plates, translucent writing on mirrors, transparencies, etc., and the process may be carried out on any hard material, such as glass, metal, Celluloid, wood and the like.

Two examples of improved articles of manufacture according to the invention are diagrammatically illustrated in the accompanying drawing, wherein:—

Figure 1 is a plan view of an advertising plaque,

65 and

Figure 2 is a section taken on the line 2—2 in Figure 1, but on an enlarged scale;

Figure 3 is a plan view showing part of a station indicator of a radio-receiving set.

Referring first to Figures 1 and 2, an advertising plaque comprises a sheet or plate of glass 10 provided on the rear face with a black legend 12 and a multicolor picture whereof the parts 14 are red and the parts 16 are black. The parts 12, 14 and 16 constituting the legend and picture may consist of powdered mineral pigment in a varnish, or in a mixture of varnish and lavender oil, provided as described above. A background 18 constituted by a gold or yellow ground coating is provided on the back of the plaque by spraying and forms a protective covering which, however, in some cases may be omitted, especially when it is desired that those parts of the plaque not covered by a picture, figure, lettering or the like shall be transparent. In Figure 2 the thickness of the layers 12, 14, 16, 18 is exaggerated for the sake of clearness.

As one example of colored sprayable mass that may be employed, 1 lb. may contain 58% mineral pigment, 30% petrol, 2% oil and 10% ink. The approximate weight of the ingredients may be:

|                 | Ounces |
|-----------------|--------|
| Mineral pigment | 9.30   |
| Petrol          | 4.8    |
| Oil             | .30    |
| Ink             | 1.6    |

The ink serves for modifying the color or tone of the powdered mineral pigment that is employed, and in some cases may be omitted.

Referring to Figure 3, the station indicator consists of a sheet or plate of glass 20 having three wave-length scales 22, 24, 26 with which the names of stations 28, 25 and 21 are respectively associated. Each scale and its associated legends are shown in a distinctive color, for example green, black and red, as indicated in the drawing. No protective coating or colored ground is provided on this indicator in order that it may be almost wholly transparent.

We claim:

A process for the photomechanical production of multi-color pictures or legends on hard material, comprising the steps of exposing to light through a transparency comprising an original to be copied, a light-hardenable coating on the hard material that contains alum in solution and exhibits a differential hardening on exposure to light, spraying a plurality of powdered mineral pigments with the aid of stencils, one for each color, which pigments are each dispersed in a fluid medium comprising approximately 10% of printer's varnish, 30% of a readily volatile liquid and 2% of oil of lavender, dusting the exposed coating with talcum powder after the colored fluid medium has been applied thereto, developing the dried colored exposed coating by removing its unhardened parts by washing with water, and removing surplus coloring matter from the developed coating.

LEOPOLD PRINZ. 65  
PAUL MORGENSTERN.